

March 27, 1928.

1,663,560

G. W. MEISTER

FILAMENT FOR INCANDESCENT LAMPS

Filed Feb. 20, 1926



INVENTOR  
GEORGE W. MEISTER  
BY  
*J. H. Gilbert*  
ATTORNEY

Patented Mar. 27, 1928.

1,663,560

# UNITED STATES PATENT OFFICE.

GEORGE W. MEISTER, OF IRVINGTON, NEW JERSEY, ASSIGNOR TO WESTINGHOUSE LAMP COMPANY, A CORPORATION OF PENNSYLVANIA.

## FILAMENT FOR INCANDESCENT LAMPS.

Application filed February 20, 1926. Serial No. 89,623.

- This invention relates to filaments for incandescent electric lamps and more particularly to a tungsten filament having a low rate of evaporation.
- 5 Blackening of the envelope of incandescent lamps, is caused chiefly by vaporization of the filamentary material and volatilization of impurities contained therein, such as carbon. The discoloration of the bulb due to vaporized impurities in the filament, is relatively slight and takes place mainly, during the initial burning of the filament. The discoloration is mainly dependent upon the vapor pressure of the filamentary material 10 and exists throughout the life of the lamp. In the case of pure molybdenum filaments, the rate of evaporation is so high as to preclude their use in incandescent lamps. Tungsten has the lowest rate of evaporation 15 of those metals which are sufficiently refractory to withstand lamp filament temperatures. However, in the case of tungsten filaments the life of the lamp and efficiency of operation are limited by the vaporization of the tungsten, resulting in decrease in the candle power of the lamp due to discoloration of the bulb.
- 20 One of the objects of the present invention is to produce a filament composed chiefly of tungsten which will have a materially lower rate of evaporation than ordinary tungsten filaments.
- 25 Another object is to provide a tungsten filament which will have a long life and high efficiency.
- 30 Another object is to provide a method of lowering the vapor pressure of a filament composed chiefly of tungsten.
- 35 Other objects and advantages will herein-  
40 after appear.
- In accordance with this invention, the tungsten filament has incorporated therewith a small percentage of another ingredient which decreases the vapor pressure of the filament and enables it to be operated at a higher efficiency than in the case of ordinary tungsten or if operated at the same temperature to give the filament a materially longer life. The additive substance 45 which I have found to be particularly effective for producing the above result, is molybdenum, when used in proportions of less than 1%. The proportion of this material which I have found to produce the best re-  
50 sult is from .05 to .25%. Higher percentages while giving a lower rate of evaporation than that of pure tungsten, do not reduce the vapor pressure to as large an extent as does the smaller proportion.
- 55 The molybdenum in the desired proportion may be admixed in powdered state directly with the powdered tungsten from which the wires are to be fabricated or if desired, reducible compounds of molybdenum and tungsten may be mixed in such proportions as to produce in the finished filament the required percentage of molybdenum. The molybdenum is employed in addition to the usual doping of thorium oxide in the case of the production of thoriated filaments or in addition to the alkali metals and other material added in the production of so-called non-sag filaments, such as covered by the patent to Pacz, 1,410,499, granted March 21, 1922, and entitled Metal 60 and its manufacture. The mixture of the powdered metals is sintered and swaged in the usual manner and drawn to the desired size.
- 65 Although I do not desire to be limited to any particular theory, it is believed that the molybdenum in small percentages, forms with the tungsten a solid solution, the vapor pressure of which is materially lower than the ordinary tungsten itself. When more 70 than 1% of molybdenum is added the excess molybdenum appears to vaporize out during burning.
- 75 In order that this invention may be more fully understood, reference may be had to the accompanying drawing the single figure of which shows a lamp adapted for determining the rate of evaporation of filaments.
- 80 This lamp comprises an envelope 1 having the filament 2 to be tested extending therethrough and connected at one end of the leading-in wire 3 and at the opposite end to a spring 4 which conducts current thereto from the leading-in wire 5. The spring 4 is adapted to apply a tension of about 5 grams in order to prevent sagging of the wire. Preferably, the bulb is formed of lime glass which has high light transmission characteristics. A glass slider 6 is loosely mounted in the envelope so as to be movable from one portion of the envelope to another, by tipping the same. The function of the slider is to protect certain parts of the envelope 85 from deposition of the tungsten vaporized 90
- 95
- 100
- 105
- 110

from the filament in order to give a comparison with those portions on which the deposition is allowed to take place. In making these tests the weight of the filament is carefully obtained before it is mounted in the lamp. The lamp is then exhausted to a high vacuum by mercury diffusion pumps and baked out at about  $400^{\circ}$  C. which temperature is maintained for 3 or 4 hours to remove as far as possible, all occluded and absorbed gases in the envelope.

An auxiliary tungsten filament is then burned in the exhaust system in order to remove water vapor from the lamp before the filament is initially lighted. The filament to be tested is then seasoned on the pumps and the lamps sealed off. A space of about 5 millimeters is marked off and each side of the center of the lamp into two zones 7 and 15 8 and the slider located so as to cover both zones. In this position the filament is seasoned for about two hours at  $2400^{\circ}$  K, to insure a thoroughly seasoned filament before starting the test. The glass slider is then 20 moved so as to expose one of the zones, as 7 while covering the zone 8. The filament is then burned at a temperature of  $2900^{\circ}$  K.  $\pm$  25  $20^{\circ}$ . At regular intervals the slider is removed from the zone 8 and readings taken 30 on both the clear portion of the envelope, i. e., zone 8 and on zone 7 on which the deposit has been allowed to take place. From these readings the temperature of the filament may be determined and the optical 35 density of the darkened portion readily ascertained.

After an optical density of from .3 to .5 is obtained corresponding to a light absorption of from 50 to 70% the lamp is broken 40 open and the filament removed and weighed to determine the loss in weight. From the loss in weight the rate of evaporation may be calculated.

It was found by these tests, which were 45 conducted with extreme care and with filaments freed as far as possible from impurities which might readily volatilize and give inaccurate results, that the molybdenum doped filaments showed a rate of evaporation much lower than that obtained with ordinary tungsten. This lowering of the rate 50 of evaporation depended upon the amount of molybdenum in the wire and appeared to

be the greatest when the percentage of molybdenum was below 1%. Very good results 55 were obtained using .25% of molybdenum.

While molybdenum has been specified as the preferred material for obtaining the desired result, it is to be understood that the invention is not so limited but any material 60 may be employed which forms solid solutions with the tungsten and lowers the vapor pressure thereof.

What is claimed is:

1. A filament for an incandescent lamp 65 consisting chiefly of tungsten and having incorporated therewith less than 1% of molybdenum, said filament having a vapor pressure lower than that of ordinary tungsten filament.

2. A filament for an incandescent lamp 70 consisting mainly of tungsten and containing from .05 to .25% of molybdenum.

3. A filament for an incandescent lamp 75 consisting of a solid solution of tungsten and molybdenum, said molybdenum being present in relatively small proportions whereby said filament has a lower vapor pressure than ordinary tungsten at the same temperature.

4. An incandescent lamp filament having 80 a low rate of evaporation composed mainly of tungsten and containing a small percentage of another ingredient which forms a solid solution therewith.

5. A filament for an incandescent lamp 85 composed chiefly of tungsten and containing less than 1% of another ingredient which decreases the vapor pressure of the filament below that of ordinary tungsten at the same 90 temperature.

6. The method of reducing the rate of evaporation of filaments composed chiefly of tungsten which consists in incorporating a small proportion of molybdenum there- 95 with.

7. The method of reducing the rate of evaporation of filaments composed chiefly of tungsten which consists in incorporating therewith less than 1% of another ingredient 100 which forms a solid solution therewith.

In testimony whereof, I have hereunto subscribed my name this 18th day of February, 1926.

GEORGE W. MEISTER.